

## UNITED STATES PATENT OFFICE

2,358,135

## MOUNTING TISSUE

Allen Abrams and George W. Forcey, Wausau, Wis., assignors to Marathon Paper Mills Company, Rothschild, Wis., a corporation of Wisconsin

No Drawing. Application November 30, 1942,  
Serial No. 467,464

7 Claims. (Cl. 117—122)

This invention relates to mounting tissue for use in affixing photographs, pictures, maps, printed matter, and the like, to any desired base by means of heat and pressure.

Heretofore, several types of mounting tissues have been available, but each of them had certain inherent characteristics which rendered them either inconvenient to use or which developed defects that vitiated their utility. For example, one type of mounting tissue consists of a dense sheet of paper coated on both sides with a heat-sealable lacquer coating. This coating is tacky under normal conditions and it is therefore necessary to interleave the mounting tissue sheets with separator or slip-sheets to prevent the sheets from sticking or blocking to each other when stacked. When such sheets are used it is necessary to remove and discard the individual separator sheets, so that the work in mounting photographs and the like is delayed by unnecessary manipulations.

Another type of mounting tissue utilizes coatings of wax compositions containing rubber. Although such coatings provide good bonds when first made, they loosen with temperature changes and also tend to weaken with age.

In accordance with the present invention we provide a mounting tissue which overcomes the disadvantages previously mentioned. Our mounting tissue is non-tacky at normal temperatures; it requires no slip-sheets to prevent blocking; it is flexible; it does not become brittle and is not affected by moisture, sunlight, or air. Our mounting tissue provides a strong adhesive bond which is not impaired by temperature changes, humidity or age. Our mounting tissue can be used for affixing photographs, pictures, maps and similar articles to any base material by heat and pressure without discoloring, staining or damaging the article mounted. Our mounting tissue obviates the need for expensive presses required for mounting articles with previous types of mounting tissues. Our mounting tissue can be used with simple inexpensive equipment, such as a hand-iron.

Our mounting tissue is made from a selected cellulosic base sheet material, which may be a dense sheet material, such as glassine, Cellophane (regenerated cellulose), or a porous type of sheet material, such as paper. We prefer to use a porous sheet material as it will carry a greater amount of bonding composition than a dense sheet and will therefore give a stronger bond.

The base sheet material is treated with a spe-

cially prepared hot-melt composition so as to provide the bonding means for affixing articles with our mounting tissue. The composition consists essentially of ethyl ether of cellulose, a plasticizer and a compatible non-volatile solvent.

The proportion of ingredients of our composition may be varied over a considerable range. The ethyl cellulose may constitute about 15 to about 50% by weight of the composition. We prefer to use ethyl cellulose having an ethoxyl content of about 40 to about 50% by weight. The plasticizer, such as hydrogenated methyl abietate, tri-phenyl phosphate, di-(para tertiary-butyl-phenyl) mono-phenyl phosphate, di-phenyl mono-(ortho-xenyl) phosphate, di-(ortho xenyl) mono-phenyl phosphate, may constitute from about 15 to about 50% by weight of the composition. The non-volatile solvent, such as hydrogenated oils, hydrogenated castor oil, and stearic acid, may be used in amounts from about 20 to about 60% by weight of the composition.

The following are specific examples of hot-melt compositions suitable for treating porous sheets, such as paper.

Table

|                                            | Percentages by weight |       |       |       |
|--------------------------------------------|-----------------------|-------|-------|-------|
|                                            | Ex. 1                 | Ex. 2 | Ex. 3 | Ex. 4 |
| Ethyl cellulose.....                       | 25                    | 20    | 20    | 40    |
| Di-(ortho xenyl) monophenyl phosphate..... | 35                    | 20    | 40    | 30    |
| Hydrogenated castor oil.....               | 40                    | 60    | 40    | 30    |

In preparing the composition, the plasticizer is first heated to about 200° F., the hydrogenated castor oil and the ethyl cellulose added, and the mixture is stirred until it is entirely free of lumps. This may require from about one to four hours, depending upon the size of the ethyl cellulose particles used. The resulting composition is clear and homogeneous and has a viscosity of about 100,000 centipoises or higher, at 200° F. as determined by Brookfield Synchro-lectric viscosimeter using 1 R. P. M. spindle speed. The molten composition is then applied in any suitable manner to both sides of the base sheet so as to distribute the composition uniformly in the sheet as well as on both its surfaces. When paper is to be treated, for example, the composition may be fed between two hot rotating rolls and the paper passed between the nip of the rolls so that both sides of the paper are coated smoothly. The treated paper is then passed over a

chilled roll to harden the composition, and it is then cut into sheets of suitable dimensions or in rolls of any desired size.

It is particularly advantageous to use a fibrous type of base sheet, such as paper, as the applied composition will penetrate the sheet which serves as a carrier for the composition. When the composition is applied to paper, we find it advantageous to have the sheet carry about 30 lbs. per ream (24 x 36—480).

Upon application of heat and pressure, our mounting tissue affixes articles securely to any suitable base, because the composition on the surface provides a direct bond between the article being mounted and the mounting tissue, as well as between the base surface to which the mounting tissue is attached. Our composition also reinforces and unifies the fibers of the base sheet so that the base sheet will not split or separate when the mounted article is subjected to a pulling force.

When a photograph, picture, map, printed matter or any desired flat sheet or article is to be affixed to any desired base, the mounting tissue, cut to suitable dimension and contour, is placed on the base, the article to be affixed is then superimposed on the mounting tissue whereupon heat and pressure are applied by any suitable means. For example, an ordinary flat-iron, heated to 250° F., is sufficient to produce an excellent bond. After mounting in the manner described, the affixed article will adhere firmly under wide extremes of ordinary temperature and humidity. The bond will not be affected by exposure to sunlight or air and it will last indefinitely. The affixed article may be removed readily from the base by merely applying heat which will soften the thermoplastic composition to permit the article to be detached intact and unimpaired.

It is to be understood that changes and modifications may be made within the scope of our invention which are intended to be included in the appended claims.

We claim:

1. A mounting tissue for photographs and printed matter comprising a cellulosic base sheet carrying a uniformly distributed hot-melt composition at both surfaces thereof comprising ethyl cellulose from about 15 to about 50% by weight, a plasticizer from about 15 to about 50% by weight and a compatible non-volatile solvent from about 20 to about 60% by weight.

2. A mounting tissue for photographs and printed matter comprising a fibrous sheet carrying a uniformly distributed hot-melt composition at both surfaces thereof comprising ethyl cellulose from about 15 to about 50% by weight, a plasticizer from about 15 to about 50% by weight and a compatible non-volatile solvent from about 20 to about 60% by weight.

3. A mounting tissue for photographs and printed matter comprising paper carrying a uniformly distributed hot-melt composition at both surfaces thereof comprising ethyl cellulose from about 15 to about 50% by weight, a plasticizer from about 15 to about 50% by weight and a compatible non-volatile solvent from about 20 to about 60% by weight.

4. A mounting tissue for photographs and printed matter comprising a fibrous sheet carrying a uniformly distributed hot-melt composition at both surfaces thereof comprising a fibrous sheet carrying a uniformly distributed hot-melt composition comprising ethyl cellulose from about 15 to about 50% by weight, an aromatic phosphate from about 15 to about 50% by weight and a hydrogenated castor oil from about 20 to about 60% by weight.

5. A mounting tissue for photographs and printed matter comprising a cellulosic base sheet carrying a uniformly distributed hot-melt composition at both surfaces thereof comprising ethyl cellulose having an ethoxyl content of about 40 to 50% by weight 25% by weight, di-(ortho xenyl) monophenyl phosphate 35% by weight, and hydrogenated castor oil 40% by weight.

6. A mounting tissue for photographs and printed matter comprising a cellulosic base sheet carrying a uniformly distributed hot-melt composition at both surfaces thereof comprising ethyl cellulose from about 15 to about 50% by weight, a plasticizer from about 15 to about 50% by weight and hydrogenated castor oil from about 20 to about 60% by weight.

7. A mounting tissue for photographs and printed matter comprising a base sheet carrying a uniformly distributed hot-melt composition at both surfaces thereof comprising ethyl cellulose (40 to 50% by weight of ethoxyl content) from about 15 to about 50% by weight, a plasticizer from about 15 to about 50% by weight and hydrogenated castor oil from about 20 to about 60% by weight.

ALLEN ABRAMS.  
GEORGE W. FORCEY.